

(Specimens.)

N. A. BUHLE.

METHOD OF ENAMELING METAL FOR JEWELRY AND  
OTHER FANCY ARTICLES.

No. 299,054.

Patented May 20, 1884.

fig. 1.



fig. 2.



WITNESSES:

*W. T. Rosenthal.*  
*Sidney Mann.*

INVENTOR

*Nicolas A. Buhle*  
BY  
*Joseph Raegner.*  
ATTORNEYS

# UNITED STATES PATENT OFFICE.

NICOLAS A. BUHLE, OF NEW YORK, N. Y.

## METHOD OF ENAMELING METAL FOR JEWELRY AND OTHER FANCY ARTICLES.

SPECIFICATION forming part of Letters Patent No. 299,054, dated May 20, 1884.

Application filed December 22, 1883. (Specimens.)

*To all whom it may concern:*

Be it known that I, NICOLAS A. BUHLE, of the city, county, and State of New York, have invented certain new and useful Improvements 5 in Methods of Enameling Metals for Jewelry and other Fancy Articles, of which the following is a specification.

This invention has reference to an improved method of enameling metals to be used for 10 dress and sleeve buttons, sign-letters, jewelry, and other fancy articles; and the invention consists in covering a suitable metallic foundation-plate with a layer of broken enamel of uniform thickness and then exposing the so- 15 covered plate to white heat, whereby the enamel liquefies and forms a uniform coating of enamel on the plate.

In the accompanying drawings, Figure 1 represents a front view, and Fig. 2 a vertical 20 transverse section on line  $yy$ , Fig. 1, of a metal plate enameled by my improved method.

Similar letters of reference indicate corresponding parts.

In carrying out my invention the surface of a 25 foundation-plate, A, of copper or other suitable metal, is first thoroughly cleaned with acids and then covered with a layer, B, of broken glass enamel, which layer is applied in uniform thickness over the entire surface of the 30 foundation-plate. The so-covered plate is

placed into a muffle and exposed to white heat in the same, by which the enamel liquefies, so that the individual particles or pieces of enamel run into each other and form a uniform coating of enamel over the entire surface of 35 the foundation-plate.

By mixing differently-colored enamels a great variety of colored effects can be obtained.

The enamel has the appearance of gayly-colored mottled ware, which can be used to advantage for various ornamental and fancy articles.

Having thus described my invention, I claim as new and desire to secure by Letters Patent— 45

The method herein described of enameling metal, which consists in covering a metallic foundation-plate with a layer of broken enamel of uniform thickness and then exposing the so-covered plate to white heat, where- 50 by the enamel liquefies and forms a uniform coating on the metal plate, substantially as set forth.

In testimony that I claim the foregoing as my invention I have signed my name in presence of two subscribing witnesses.

NICOLAS A. BUHLE.

Witnesses:

PAUL GOEPFEL,  
SIDNEY MANN.